

(No Model.)

H. Y. CASTNER.

PROCESS OF MANUFACTURING SODIUM AND POTASSIUM.

No. 452,030.

Patented May 12, 1891.



Witnesses:

H. S. McArthur  
J. A. Fairgrieve.

Inventor:

Hamilton Young Castner  
By Foster Freeman  
Attest

# UNITED STATES PATENT OFFICE.

HAMILTON YOUNG CASTNER, OF LONDON, ENGLAND.

## PROCESS OF MANUFACTURING SODIUM AND POTASSIUM.

SPECIFICATION forming part of Letters Patent No. 452,030, dated May 12, 1891.

Application filed September 3, 1890. Serial No. 363,856. (No specimens.)

To all whom it may concern:

Be it known that I, HAMILTON YOUNG CASTNER, a citizen of the United States of America, residing at No. 115 Cannon Street, in the city of London, England, have invented an Improved Process for the Manufacture of Sodium and Potassium; and I do hereby declare that the following is a full, clear, and exact description of the invention, which will enable others skilled in the art to which it appertains to make and use the same.

This invention relates to a process for the production of sodium or potassium from caustic soda or potassa without distillation, where-  
15 by the cost of production is considerably re-  
duced. Briefly stated, the process may be  
said to consist in submitting fused caustic  
alkali maintained at a low temperature to  
the decomposing action of the electric cur-  
rent, suitable apparatus being provided for  
20 collecting the separated metal. I am aware  
that so long ago as 1808 Sir Humphrey Davy  
electrolyzed caustic soda and produced the  
alkaline metal in a minute quantity; but the  
25 method adopted in such experiment did not  
enable the metal to be commercially produced,  
and I believe that prior to my present invention  
it was not known that only under cer-  
tain conditions of temperature could the elec-  
30 trolysis be effected, as I have failed to find  
that any process has heretofore been sug-  
gested for commercially manufacturing the  
alkaline metals, either by chemical or elec-  
trical means, that did not involve the use of  
35 a temperature sufficient to insure the distil-  
lation of the metal. All such processes are  
more or less wasteful, owing to the loss of  
material and to the wear and tear of the ap-  
paratus consequent upon the high tempera-  
40 tures necessarily employed. My experiments  
have proved that to secure any practical re-  
sult from the electrolysis of either caustic  
soda or potash it is absolutely necessary that  
the temperature be kept as low as possible  
45 while insuring the liquidity of the electrolyte.  
At their melting-points both caustic soda and  
caustic potassa while being electrolyzed re-  
combine in a degree both with the alkaline  
metal and oxygen, and at even slight eleva-  
50 tions of temperature this recombining power  
rapidly increases and finally becomes so great  
at higher temperature that the products from

the electrolysis are recombined as rapidly as they are formed and practically no decom-  
position is obtained. Thus I have found that 55  
in order to attain any practical result such  
means must be employed as will insure a con-  
stant and low temperature, while at the same  
time the elements produced from the decom-  
position should be given an opportunity of 60  
escaping or being removed from the absorbing  
power of the electrolyte as quickly as  
possible. In carrying out my present invention  
there is practically no waste or loss of  
material, while the wear and tear upon the 65  
apparatus are small.

In order that others skilled in the art may  
fully comprehend my invention, reference is  
made to the accompanying drawing, which  
represents a sectional elevation of a conven-  
70 ient form of apparatus for carrying my in-  
vention into effect.

Said apparatus consists of an iron vessel or  
receptacle A, suitably mounted in brick-work  
R, so that the heat applied by the gas-burn-  
ers G may be well distributed. The vessel  
A is provided with one or more base pipes or  
75 extensions B, adapted to receive the negative  
electrodes H, which are preferably of metal  
and pass up into the vessel. Suspended di-  
rectly above the said cathode is a tubular iron  
80 receptacle or vessel C, which is provided on  
its upper end with a lid N, and to its lower  
edges is secured an iron-wire-gauze cylinder  
M, the said gauze, when the receptacle N is 85  
placed in position, completely surrounding  
the cathode. The positive electrodes F are  
preferably made of such metal as will with-  
stand the oxidizing action of the evolved  
gases and either form part of the cover of the 90  
vessel A or may be bolted thereon, being so  
placed that when the cover is adjusted the  
electrodes are a suitable distance from and  
directly surround the gauze M. Electrical  
connection is made between the cover by the 95  
connection I with the positive pole of the dy-  
namo and by the connection L with the neg-  
ative pole. The cover is provided with an open-  
ing P for the escape of gases resulting from  
the electrical action, this opening also serving 100  
for the introduction of a thermometer or other  
heat-registering device. Insulation is made  
at the points S S by means of asbestos or  
other insulating medium. The size and dis-

tance apart of the electrodes are both proportioned to the quantity of current to be supplied. Should the electrodes have a larger surface than is actually required, the elements 5 set free at each electrode are exposed to the absorbing-alkali to a greater extent than necessary and a quantity of the electrical action is wasted, owing to the elements being absorbed and recombining. Should the electrodes 10 be too small, the resistance will be increased to such an extent that the bath will be unduly heated and that at the very points where an excess of temperature is most objectionable. As an example, the drawing filed 15 herewith is made to scale and illustrates an apparatus which I have found practicable, and in which the negative electrode H is four inches in diameter, and the vessel is adapted to contain a bath of two hundred and fifty 20 pounds of molten caustic alkali. This apparatus is adapted for use with a current of about twelve hundred ampères in strength. If a suitable electric current be passed through the molten caustic soda or potash E, the alkali 25 being kept at a very low temperature—say within 20° centigrade of its melting-point—any water contained in the caustic will be decomposed first and resolved into its elements of hydrogen and oxygen, which will be given off at the negative and positive electrodes, respectively. When this action has 30 ceased, the current will act upon the caustic alkali, oxygen or a mixture of oxygen and water being given off at the positive pole, 35 while the alkaline metal and hydrogen or the alkaline metal alone are given off at the negative pole.

In the apparatus as described the alkaline metal, (being much lighter than the caustic,) 40 together with the hydrogen, will rise from the negative electrode and pass into the receiver C, the hydrogen escaping around the edges of the cover N, while the molten metal continues to collect in quantity. From time to 45 time this collected metal D is removed by means of a large finely-perforated spoon, the perforations enabling the molten caustic to flow out, while the metal remains in the spoon. Caustic is added to the bath from time to 50 time to replace the metal removed, and in this manner a continuous process may be carried on without the aid of an expensive plant and in an economical manner. As before mentioned, any increase of temperature is followed by a 55 proportionate loss of product and waste of

electrical energy; but it is possible to so adjust the electrical current and the quantity of caustic alkali forming the electrolyte that the proper temperature will be maintained in a previously-melted bath without external heat 6 or even by an increase of current to melt the bath, subsequently reducing the quantity of current until the working temperature is attained.

The cathode may be conveniently sealed in 6 the extension B by means of molten caustic K, which is allowed to harden before beginning the process.

In order to secure a fair yield of alkaline metal for the current applied, it is necessary 7 that the temperature of the electrolyte should not be allowed to go above 20° centigrade of the respective melting-points of the caustic used, yiz: In using caustic soda, having a melting-point of about 310° centigrade for the 7 electrolyte the temperature should be maintained below 330° centigrade. The same rule is to be observed in respect to the caustic potash or to a mixture of the two hydrates, the same having a lower melting-point than either 8 the potash or soda compound alone.

I do not of course confine myself to the particular form of apparatus shown, but simply describe it as one of the forms which may be employed. 8

Having now particularly described and ascertained the nature of my said invention and in what manner the same is to be performed, I declare that what I claim is—

1. The hereinbefore-described process of 9 manufacturing the alkaline metals, which consists in treating the caustic alkali while constantly maintained at a temperature of not more than 20° centigrade above its melting-point to the action of the electric current, 9 substantially as described.

2. In an apparatus for the manufacture of alkaline metals, the combination, with positive and negative electrodes, of the gauze or screen interposed between said electrodes and a superposed vessel or dome for collecting the separated metal, substantially as set forth. 1

In testimony whereof I have hereunto set my hand in the presence of two subscribing witnesses.

HAMILTON YOUNG CASTNER.

Witnesses:

PHILIP M. JUSTICE,  
WILLIAM TRIMMER.